

Jan. 29, 1963

H. E. SPOONER

3,075,281

METHOD FOR PRODUCING AN ELECTRICAL CONTACT ELEMENT

Filed Oct. 3, 1958

**FIG. 2**



**FIG. 1**



**FIG. 3**



**FIG. 4**



**FIG. 5**



INVENTOR.

HOWARD E. SPOONER

BY

*Karl Huber*  
*James E. Bryan*  
ATTORNEYS

1

3,075,281

## METHOD FOR PRODUCING AN ELECTRICAL CONTACT ELEMENT

Howard E. Spooner, Lincoln, R.I., assignor, by mesne assignments, to Engelhard Industries, Inc., Newark, N.J., a corporation of Delaware

Filed Oct. 3, 1958, Ser. No. 765,234

2 Claims. (Cl. 29—155.55)

This invention relates to a method for producing an electrical contact element and, more particularly, is concerned with a method which permits the insertion of contact points of precious metal into a supporting base metal strip, the surface of the contact point contacting a base metal oxide.

It is known that the properties of precious metal contacts are improved by additions of base metal oxides or mixtures thereof such as iron, cobalt, nickel, copper, cadmium, chromium, manganese, tin and many others. The contacts produced from precious metals with added base metal oxides show a decreased tendency to stick during performance and are used in a great number of applications. However, one of the main difficulties encountered with this type of contact resides in the fact that the base metal oxide addition renders the material unsolderable and numerous methods exist to secure such contact points in supports. On the other hand, in U.S. Patent No. 2,625,737, a method has been described in which precious metal contacts are obtained by preparing a disc from a laminated stock sheet metal having a top layer of a precious metal. Subsequently, the disc is inserted into an aperture in a base metal strip, the aperture having a shape substantially identical with that of the disc, the strip serving as the support for the contact. The disc is bonded to the walls of the aperture and finally bent outwardly from the plane of the support, in order to form a raised contact point.

It has been found that this method, as described in U.S. Patent No. 2,625,737, can be successfully employed to produce electrical contact elements having a contacting surface of precious metal admixed with a base metal oxide. This invention therefore constitutes a further development of the method described in the aforementioned U.S. patent, thereby combining the advantages of precious metal contacts with added base metal oxides and those of the known method. Slight modifications of the method have been found useful, as described below.

In accordance with the invention, an electrical contact element, having at least one contact point of a precious metal with an added base metal oxide and being mounted in a supporting base metal strip, is obtained by forming a disc from a laminated metal sheet having two layers, bonded to each other, the first layer consisting of a precious metal containing a metal oxide whereas the second layer consists of any precious or base metal capable of being bonded to the desired support by means of a heat treatment, the second layer having a melting point not higher than that of the first layer. Good results have been obtained when using silver. Subsequently, the disc is inserted into an aperture in the support, of substantially identical shape to that of the disc, whereupon the assembly is subjected to a heat treatment in order to bond the sides of the second layer of the disc to the adjacent portions of the walls of the aperture. A raised contact point is finally obtained by bending the bonded disc outwardly from the plane of the adjacent portions of the support by means of dies and pressure.

In the following, the invention will be described in connection with contacts of fine silver with added base metal oxide, without being restricted thereto, and by reference to the accompanying drawing in which one

2

embodiment of the invention is illustrated. In the drawing

FIGURE 1 is a section through a laminated disc,

FIGURE 2 is a fragmentary section through the supporting base metal strip,

FIGURE 3 is a fragmentary section through the base metal strip of FIGURE 2 having a disc of FIGURE 1 inserted therein,

FIGURE 4 is a section through a finished contact element, and

FIGURE 5 is a section through a punch press suitable for applying the method of the invention and illustrating the combined steps of forming the disc and inserting the disc into the supporting strip.

15 The method of the invention is intended to be used especially in connection with silver contacts having a base metal oxide added to the contact surface and therefore will be described in connection therewith, without being limited to silver contacts. Referring to FIGURE 1, a disc 8 is provided which consists of a bottom layer 10 of silver having a top layer 12 of silver thereon with which a selected base metal oxide is in admixture. For the purpose of mass production, the discs 8 are blanked out from laminated sheet metal stock, as described hereinafter in connection with FIGURE 5. However, when desired, the top layer may be a layer of silver containing a metal capable of forming an oxide and the oxidation of this metal can be effected at any time during the process and even after the contact element is finished.

30 FIGURE 2 illustrates the base metal strip 14 forming the support for the contact and which is fabricated from any desired material such as copper, brass or the like. At the location where the contact is to be inserted, the strip 14 is provided with an aperture of a shape substantially identical with that of the disc, generally in the form of a circle. Subsequently, the disc 8 is inserted into the aperture as shown in FIGURE 3 and subjected to a heat treatment in a furnace at a temperature within or above the softening range of silver, whereby the wall 40 16 of the layer 10 of the disc is firmly bonded to the adjacent portion of the wall 18 of the aperture in the support 14. No bonding occurs between the comparatively narrow edge of the layer 12 and the adjacent portion of the aperture wall 18 since this layer contains 45 a base metal or a base metal oxide but it has been found that, for all practical purposes, when making the layer 10 sufficiently thick, a firm bonding between the disc 8 and the support 14 is obtained. Especially when using silver, the bond is strong enough to permit the final shaping effected by die pressing and illustrated in FIGURE 5, where the disc 8 is bent outwardly from the plane of the adjacent portion 20 of the support to form a raised contact point.

55 In the aforementioned U.S. Patent No. 2,625,737, the disc described therein has a third layer on its bottom consisting of a solder, which is partly drawn up around the sides of the disc when the disc is punched out from the laminated metal stock, and serves to accomplish the bond. Such a solder layer may be used in connection 60 with the present invention as well, but it has been found that, when the layer 10 is made from a metal having a melting point not higher than that of the first layer, e.g. silver, no solder is required and a sufficiently strong bond is obtained.

65 Referring to FIGURE 5, a die press suitable for manufacturing contacts in accordance with the invention consists of a die 22 passing through a guide plate 24 and cooperating with a die plate 26 having a bore 28 therethrough, the diameter of the bore 28 corresponding to 70 the diameter of the disc 8 punched out by the device. A laminated metal sheet consisting of a layer 10 of pure silver and a second layer 12 of silver combined with the

base metal oxide and bonded to the pure silver layer is passed between the guide plate 24 and the die 26. Simultaneously, the base metal strip 14 forming the support is passed through a recess 30 in the lower surface of the die 26 in such a way that the aperture 18 is aligned with the bore 28. The punch 22, when moving downwardly, punches out the disc 8 and immediately inserts the disc into the aperture in the supporting strip 14 in one operation. The strip 14 carrying one or more discs 8 within one or more apertures is subsequently introduced into a furnace and heated to a temperature suitable to insure the bond between the layer 10 of the disc 8 and the wall 18 of the apertures in the strip 14. Finally, the contact elements are blanked out from the strip 14 and shaped by suitable die pressing to the form shown in FIGURE 4, for example, by bending over the edges of the strip 14 as shown at 32 and 34 and by displacing the initial disc 8 outwardly from the plane of the surrounding portions 20.

It has been pointed out above that the base metal oxide can be incorporated into the top layer 12 of the laminated stock before blanking out the discs 8. However, good results have been obtained when using a layer 12 made from silver and containing a base metal capable of forming an oxide whereby the formation of the oxide in the layer can be effected at any moment during the process of manufacturing the contact and even when the contact element is finished. In any event, a strong bonding of the side wall 16 of the layer 10 to the adjacent portions of the wall 18 of the aperture will be obtained, which results in a precious metal contact surface containing a base metal oxide supported by a base metal strip, without the necessity of soldering the oxide-containing material.

It will be obvious to those skilled in the art that many modifications may be made within the scope of the present invention without departing from the spirit thereof, and the invention includes all such modifications.

What is claimed is:

1. A method for producing an electrical contact element having at least one contact point of silver containing a base metal oxide and mounted in a base metal support, which comprises forming a disc from a laminated metal sheet having first and second layers bonded to

each other, the first layer consisting essentially of a thin layer of silver in admixture with an oxide of a base metal selected from the group consisting of iron, cobalt, nickel, copper, cadmium, chromium, manganese, tin and admixtures thereof, the second layer consisting essentially of a comparatively thicker layer of silver; inserting the disc into an aperture in said support; bonding the side wall of the second layer of the disc directly to the adjacent wall of the aperture by means of a heat treatment; and displacing the bonded disc outwardly from the plane of the support to form a raised contact point.

2. A method for producing an electrical contact element having at least one contact point of silver containing a base metal oxide and mounted in a base metal support, which comprises forming a disc from a laminated metal sheet having first and second layers bonded to each other, the first layer consisting essentially of a thin layer of silver in admixture with an oxidizable metal selected from the group consisting of iron, cobalt, nickel, copper, cadmium, chromium, manganese, tin and admixtures thereof, the second layer consisting essentially of a comparatively thicker layer of silver; inserting the disc into an aperture in said support; bonding the side wall of the second layer of the disc directly to the adjacent wall of the aperture by means of a heat treatment; and displacing the bonded disc outwardly from the plane of the support to form a raised contact point; the method also including oxidizing at least a portion of the oxidizable metal content in the first layer.

#### References Cited in the file of this patent

#### UNITED STATES PATENTS

|           |             |               |
|-----------|-------------|---------------|
| 2,148,040 | Schwarzkopf | Feb. 21, 1939 |
| 2,226,944 | Reeve       | Dec. 31, 1940 |
| 2,360,522 | Shobert     | Oct. 17, 1944 |
| 2,365,249 | Comstock    | Dec. 19, 1944 |
| 2,373,861 | Van Inwagen | Apr. 17, 1945 |
| 2,382,338 | Shobert     | Aug. 14, 1945 |
| 2,425,052 | Swinehart   | Aug. 5, 1947  |
| 2,425,053 | Swinehart   | Aug. 5, 1947  |
| 2,625,737 | Spooner     | Jan. 20, 1953 |
| 2,861,155 | Farnham     | Nov. 18, 1958 |